

C. PACK.  
CASTING PROCESS.  
APPLICATION FILED JAN. 13, 1919.

1,302,958.

Patented May 6, 1919  
2 SHEETS—SHEET 1.



INVENTOR.  
*Charles Pack*  
BY  
*J. Edwards*  
ATTORNEYS.

C. PACK.  
CASTING PROCESS.  
APPLICATION FILED JAN. 13, 1919.

1,302,958.

Patented May 6, 1919.  
2 SHEETS—SHEET 2.

Fig. 7.



Fig. 8.



Fig. 9.



Fig. 10.



Inventor  
Charles Pack  
By his attorney  
P. Edwards

# UNITED STATES PATENT OFFICE.

CHARLES PACK, OF BROOKLYN, NEW YORK, ASSIGNOR TO DOEHLER DIE CASTING COMPANY, OF BROOKLYN, NEW YORK, A CORPORATION OF NEW YORK.

## CASTING PROCESS.

1,302,958.

Specification of Letters Patent.

Patented May 6, 1919.

Application filed January 13, 1919. Serial No. 270,817.

To all whom it may concern:

Be it known that I, CHARLES PACK, a citizen of the United States, residing at the borough of Brooklyn, in the city of New York, county of Kings, and State of New York, have invented certain new and useful Improvements in Casting Processes, of which the following is a specification.

My invention relates to processes involved in casting tubular objects which have bent or offset or curved portions, such that it would be impossible to cast the same about cores, by the usual methods, and then withdraw the cores. For example, in the case 10 of a hollow tube having its end portions bent at right angles to its main body portion, it would be manifestly impossible to cast or mold the same, as an integral construction, about three cores, and then withdraw all of the cores in the usual manner, because there would be no way of getting out the core for the main body portion. In such a case, in accordance with my invention, the core which by the usual practice 15 could not be removed, is allowed to extend out through the die or mold, and thus form a hole or opening in what should be one of the finished walls of the object being cast. When the casting has been poured, the cores 20 are withdrawn, and the edges of the hole or opening referred to are coated with a solder, after which the object is again placed in a suitable die, and a core inserted in the nearest end, so as to cover the hole or opening 25 referred to. Metal may now be poured into the die or mold and against the core, so as to fill up the hole or opening and make an integral structure with the original casting, having no perceptible joint. The same 30 general process may be used in various situations, as for example, in case it is desired to cast a tubular body having a curved surface at the intersection of two portions which are disposed at an angle to each 35 other. In such a case the curved surface may be formed by an extra core, which is withdrawn through an opening which is later tinned or soldered and then filled up, by the aid of an additional core, in the 40 manner described above.

In order that a clearer understanding of my invention may be had, attention is hereby directed to the accompanying drawings, forming part of this application, and illus-

trating certain ways in which my invention may be carried out. In the drawings, Figure 1 is a plan view of a die showing what may be termed a tone arm in process of formation therein, in cross section, with three core pins in position; Fig. 2 is a cross section taken on line 2-2 of Fig. 1; Fig. 3 is a partial plan view of the tone arm shown in Fig. 1; Fig. 4 is an end view of the same; Fig. 5 is a plan view similar to Fig. 1 showing a further step in the process; Fig. 6 is a front elevation partly in cross section of the completed object formed in the preceding figures; Fig. 7 is a plan view of a die or mold showing a modified form of construction being cast, the object 50 being cast being shown in cross section; Fig. 8 is a similar view showing a further step in the process; Fig. 9 is an end view corresponding to the operation indicated in Fig. 8; and Fig. 10 is a front elevation partly shown in section of the completed object.

Referring first to the form of my invention indicated in Figs. 1 to 6 inclusive, I have indicated the casting of a hollow tubular arm having a main tapering horizontal portion 1 and a pair of end portions 2 and 3 which are offset at right angles from the portion 1. Obviously, if it were attempted to cast this object as an integral construction about three cores, it would be impossible to withdraw the core about which the portion 1 was cast. In accordance with my invention a core 4 is used to form the main portion 1 of the tone arm or tubular object 50 to be cast, this core extending out of the die 5 to the left. Straight cores 6 and 7 are used to form the end portions 2 and 3 of the tone arm, in the usual way. The cores being properly positioned in the mold 55 cavities of the die, the metal is poured, with the result that the object is completely formed about the three cores, except for the fact that there is a hole or opening 8 formed at the end of the portion 1 of the object 100 above the offset end 6 thereof, through which hole the core 4 extends. The metal having been poured the cores are withdrawn, the core 4 being withdrawn through the opening 8.

The edges of the opening 8 are now given a light coating with a molten soldering or tinning mixture and the object placed in an-

other die 5' with another core 9 inserted in the end 2 of the object. This core 9 has its inner end suitably formed to press against the surface of the tone arm in which the hole 8 appears. The die 5' being suitably gated, as shown at 5", molten metal is poured therein against the end of the core pin 9 to a sufficient extent to fill the opening 8 and make an integral construction therewith. When the metal has sufficiently solidified, the core pin 9 is withdrawn and the opening 8 will be found to have been completely filled so that an integral construction is presented in which no joint is apparent after a slight polishing or finishing of the article.

A further application of the principle is illustrated in Figs. 7 to 10 inclusive of the drawings. Ordinarily when a hollow elbow or other tubular object having portions which meet at an angle is cast, it is necessary that the angular portions should intersect with a straight line joint because of the necessity of withdrawing the core pins in straight lines. By practising my invention, however, it is possible to produce any desired curved surface at the intersection of the angular portions of such a construction.

As shown in Figs. 7 to 10 an elbow 10, for example, may be constructed having end portions 11 and 12 which extend substantially at right angles to each other and are joined together by a gradual smooth curve on both the inner and outer sides of the angle. This may be accomplished by the use of a suitable die 13 in which are located a pair of straight core pins 14 and 15 which are adapted to form the straight end portions 11 and 12 of the construction. I also make use of an additional core pin 16 which is inserted at an angle into the die or mold between the core pins 14 and 15, the ends of which are positioned to abut against the peripheral surfaces of the pin 16. The inner end of the core pin 16 is suitably curved to form the desired curved surface 17 at the inner side of the elbow, at the intersection between the two straight end parts of the elbow.

The core pins being arranged as described the molten metal is poured after which the core pins 14, 15 and 16 are withdrawn, the pins 14 and 15 being withdrawn through the ends of the elbow in the usual manner while the pin 16 is withdrawn in the direction of its length through the opening 18, which is formed in the outer curved surface of the elbow by the extension of core pin 16 through the same. The edges of the opening 18 may now have a light film of molten metal, such as a suitable soldering or tinning composition placed on the same, after which the elbow is positioned in a suitable die 13' and an additional core pin 19 is in-

serted through the straight end portion 11 of the elbow into position to press against the inner surfaces of the part in which the opening 18 is formed, as is indicated in Fig. 8. Molten metal is then poured into the die 13' through a suitable gate so as to fill the opening 18 and complete the structure of the elbow, as is shown in Fig. 10, the opening 18 being smoothly filled with metal so as to form an integral construction with the remainder of the elbow without any apparent joint. When the metal has sufficiently solidified, the core pin 19 is withdrawn.

The drawings illustrating my invention are, of course, somewhat diagrammatic, it not being deemed essential, for example, to illustrate the manner in which the dies are gated. When the opening 8, as shown in Figs. 3 and 4, and the opening 18, as shown in Fig. 9, are to be filled up, the dies 5' and 13' in which the objects are placed may conveniently be gated at points adjacent to the openings which are to be filled up as described. My process is particularly adapted for the manufacture of finished castings by the pressure die casting method. It will be obvious that my invention is not limited in its applicability to the constructions described and illustrated, these latter being merely given for purposes of illustration and exemplification.

What I claim is:

1. A method of casting a tubular object, consisting in first casting such an object complete save at a point at which an opening in the object is left, and then casting a closure for said opening. 100

2. A method of casting a tubular object, consisting in first casting such an object complete save at a point at which an opening in the object is left, treating the edges of said opening, and then casting a closure for said opening. 105

3. A method of casting a tubular object, consisting in casting such an object about one or more cores, one of which extends through what will be a closed surface of the finished object, drawing the core or cores, and then casting a closure for the opening left by the withdrawal of said extended core. 110

4. A method of casting a tubular object, consisting in casting such an object about one or more cores, one of which extends through what will be a closed surface of the finished object, drawing the core or cores, 120 inserting another core within the object to cover the opening left by the withdrawal of said extended core, and casting a closure for said opening against said last named core.

5. A method of casting a tubular object, 125 consisting in casting such an object in a die or mold with the aid of one or more cores, one of which extends through what will be a closed surface of the finished object, drawing the core or cores, applying molten metal 130

to the edges of the opening left by the withdrawal of said extended core, and then casting a closure for said opening.

6. A method of casting a tubular object having bent or curved portions, consisting in so locating a plurality of cores in a die, in an angular relation, as to form a desired section, with an elongated one of the same extending through what will be a closed surface of the finished object, pouring molten metal around said cores in the die, drawing the cores, inserting another core into the object to cover the said opening, pouring molten metal against said core to fill said opening and complete the structure of the object, and withdrawing said core.
7. A method of casting a tubular object having bent or curved portions, consisting in so locating one or more cores in a die, that the same may subsequently be withdrawn in straight lines from end or other desired openings of the finished object, and so locating another core that the same extends through what will be a closed surface of the finished object, pouring molten metal around said cores in the die, to form the complete object except for the temporary opening through which said last named core extends, drawing said cores, and filling said temporary opening with metal to complete the structure of the object.

8. A method of casting a tubular object having bent or curved portions, consisting in so locating two or more cores in a die as to form a desired section, with one of the same extending from what will be an end or other opening of the finished object, and

with an adjacent one of said cores extending through what will be a closed surface of the finished object, pouring molten metal around said cores in the die, drawing the cores, placing molten metal on the edges of the opening through which said second core was withdrawn, placing the object in a suitable die, inserting a core through an end or other opening thereof to cover the said opening through which the second core was withdrawn, pouring molten metal against said core in the die to close said opening and complete the structure of the object, and withdrawing said core.

9. A method of casting a tubular object having straight portions at an angle to each other connected by a curved surface, consisting in positioning cores in a die to form the straight portions, and a third core between the same in position for its end surface to form the desired curved surface of the object, said core extending through what will be the wall of said object opposite to said curved surface, pouring molten metal around said cores in the die, drawing the cores, placing the object in another die with a core inserted through one of said straight portions to cover the opening through which said third core was withdrawn, pouring molten metal against said core to fill said opening and complete the structure of the object, and withdrawing said core.

This specification signed and witnessed this 7th day of January, 1919.

CHARLES PACK.

Witnesses:

FRED C. STOLTING,  
EDMUND J. WARD.